

# UNITED STATES PATENT OFFICE.

FRANÇOIS HYRONIMUS, OF CUGNY, FRANCE.

## CHARGING OF PRIMERS.

No. 908,674.

Specification of Letters Patent.

Patented Jan. 5, 1909.

Application filed February 4, 1908. Serial No. 414,282.

*To all whom it may concern:*

Be it known that I, FRANÇOIS HYRONIMUS, a citizen of the French Republic, and resident of Cugny, Seine et Marne, France, have 5 invented new and useful Improvements in the Charging of Primers, of which the following is a specification.

This invention has reference to a new primer for the ignition of mines or for igniting 10 the charges of fire-arms.

For some time trials have been made to substitute the fulminate of mercury by different explosives or explosive mixtures which are cheaper, simpler to prepare and of 15 at least equal efficacy. Up to the present the only progress which seems to have been effected in the charging of primers for mines has been the substitution for the pure fulminate of a mixture of fulminate with an 20 oxidizer, such as for example chlorate of potassium, or of a primer consisting of a charge of an organic nitrated substance (picric acid, trinitrotoluene, and the like) which itself is primed through pure fulminate used 25 in small quantity only. The different mixtures used for the primers for fire-arms all contain fulminate of mercury in quantities varying according to requirement, and the addition of other substances merely serves 30 for modifying the flame and for regulating the sensitiveness with regard to shocks or friction.

The object of the present invention is to replace the fulminate of mercury wherever it 35 may be employed by trinitrid of lead  $(\text{Az}_3)_2\text{Pb}$ . This compound whose properties have hitherto not been generally known is found to possess the same explosive qualities as the fulminate of mercury, that is to say, its 40 explosion, if effected in a suitable manner (by shock, ignition, etc.) produces an energetic molecular vibration which is adapted to detonate the usual explosives, such as dynamite, explosives of the Favier type, gun-cot- 45 ton etc.

The preparation of the trinitrid of lead is very simple and without danger when proceeding in the manner hereinafter described. The amid of sodium is prepared in the classical manner by sending through melted sodium a jet of dry ammonia gas. This amid is treated with a jet of dry protoxid of nitrogen at a temperature of  $300^\circ\text{C}$ ; the amid in fusion is transformed into trinitrid of sodium

which is solid at the temperature at which one operates.

The trinitrid of sodium, when cooled, is absorbed by the water; the solution obtained is alkaline. It is exactly neutralized with highly diluted nitric acid and to the neutral solution is added a solution of nitrate of lead. The trinitrid of lead precipitates in crystals, the size of which varies with the temperature at which the double decomposition is effected. These reactions 65 take place according to the following formulae:—



70

The water which is formed with this reaction decomposes part of the amid according to the formula:—



75

The double decomposition is the following:—



The crystalline precipitate of  $(\text{Az}_3)_2\text{Pb}$  is collected on a filter, washed out with cold 80 water and dried at a temperature below  $100^\circ\text{C}$ . It is now ready to serve for the charging of any primers, exactly in the manner as the fulminate of mercury.

For industrial purposes and with a view 85 to obtaining a convenient output, the theoretical process which has just been described, will be applied as hereinafter described.

The trinitrid of sodium infusible at the temperature of  $300^\circ\text{C}$ . at which the operation 90 is carried on, the amid being however fusible at this temperature, the nitrous oxid therefore will only with difficulty react when a certain quantity of trinitrid has formed and it absorbs the amid not yet decomposed. 95 This fact retards the operation and causes a much larger quantity of nitrous oxid to be used than is really required. To obviate this inconvenience, it is necessary to divide the amid of sodium in having it partly ab- 100 sorbed by an infusible material, which is anhydrous, porous and which does not react with the different substances intervening in the reaction. Pumice-stone, infusorial earth, etc., cannot be used for this purpose owing 105 to their silicious nature; the sodium-hydrate which is formed, would react upon the silicic material, whereby the reaction would

become even more difficult, the output being at the same time much reduced. There have to be chosen anhydrous materials, such as lime, magnesia, sulfate of soda, etc., which fulfil the required conditions.

The operation is as follows:—The lime, for example, is crushed; further the amid is crushed and the two materials are placed in a suitable receptacle so that the mixture is spread over a large surface; the receptacle is heated to a temperature of at least 190°C.; the amid, in melting, is absorbed by the lime so that the nitrous acid easily penetrates into the material and operates its reaction. Mechanical kneading may be used. The mass obtained is lixiviated with water and treated as has been described.

The trinitrid of lead, although it has already been prepared in laboratories in very small quantities, has up to the present never found commercial application.

The experimentists who have studied the

application of hydrozoic acid and its salts to explosives, have had some accidents which apparently have prevented them from continuing their experiments.

The process of manufacture hereinbefore described is absolutely secure and the dry trinitrid of lead, when ready for use, is not more difficult to manipulate than the fulminate of mercury, for which it is substituted.

It is to be understood that the present invention does not concern any other applications or properties of this material, but merely its special explosive qualities.

I claim:—

A primer for mines and fire-arms consisting of a charge of trinitrid of lead.

FRANÇOIS HYRONIMUS.

Witnesses:

H. C. COXE,  
ALFRED FREY.